

A. BONTEMPI.

RUST PROOFING IRON, STEEL, OR THE LIKE.

APPLICATION FILED AUG. 11, 1911. RENEWED MAY 16, 1913.

1,072,904.

Patented Sept. 9, 1913.

Fig. 2.



Fig. 1.



Witnesses:

Chalco C. Cass  
L. H. Grote

Inventor  
AUGUSTO BONTEMPI  
By his Attorneys  
Thomas and Norman

# UNITED STATES PATENT OFFICE.

AUGUSTO BONTEMPI, OF NEW YORK, N. Y., ASSIGNEE TO BONTEMPI RUST PROOFING COMPANY, A CORPORATION OF NEW YORK.

## RUST-PROOFING IRON, STEEL, OR THE LIKE.

1,072,904.

Specification of Letters Patent.

Patented Sept. 9, 1913.

Application filed August 11, 1911, Serial No. 643,581. Renewed May 16, 1913. Serial No. 766,158.

*To all whom it may concern:*

Be it known that I, AUGUSTO BONTEMPI, a subject of the King of Italy, and residing in the city, county, and State of New York, have invented certain new and useful Improvements in Rust-Proofing Iron, Steel, or the Like, of which the following is a specification.

This invention relates to the process of rust proofing metal surfaces and has for its object not only to expedite the process but also to protect the metal article treated from heat injury during the process.

In the rust proofing process hitherto described by me in Patent 881,221, the temperature of the chamber in which the metal is placed during treatment is stated to be raised to from 1000° F. to 1800° F. and the metal thus heated is subjected for several hours to the action of the fumes of suitable non-corrodible material which is fused and the fumes from which enter the pores of the highly heated metal as a gas and penetrate to a greater or less depth, serving on cooling to form a non-corrodible surface on the metal. The temperature of the article under treatment was kept high enough during treatment to insure the maintenance of the fumes of the non-corrodible material in gaseous condition during treatment. In practice it has been found that the maintenance of the article under treatment at a temperature sufficiently high for this purpose results frequently in serious injury to the article, and the utility of the process was thus limited to articles of such character that the high temperature at which they were kept in the treating chamber did not injuriously affect the same, while at the same time the duration of the treatment was necessarily prolonged to an undesirable extent.

I have now found by further experimentation that the process is greatly expedited and the article under treatment safe-guarded against heat injury if its temperature be kept below that at which the rust proofing material fumes so that the fumes of the rust proofing material introduced into the treating chamber condense at once upon the article under treatment. At the same time, the article should be heated to such temperature that the pores of the metal are suitably opened to receive the condensed material and preferably the article is heated to

a sufficient temperature to maintain the condensed rust proofing material in fused condition thereon during the continuance of the treatment. Upon cessation of the treatment and the cooling of the article, the rust proofing material hardens into a durable and efficient rust proofing surface, the thickness of which depends, of course, upon the length of the treatment. In ordinary cases the treatment is complete at the end of from half an hour to two hours treatment.

When treating iron the desired effect is obtained by heating the same to approximately from 900° to 1200° F. in a muffle chamber to which is led the fumes of a fused non-corrodible substance or compound which condense in fused condition at this temperature. The compounds used by me fume at a temperature of approximately 1400° F. so that the fumes therefrom which are introduced into the treating chamber or muffle at this temperature condense rapidly upon the articles therein which are maintained at the lower temperature of 900° to 1200° F. Before subjecting the iron to the action of these fumes it may be treated with superheated steam, as I have previously suggested, and this is advantageous with heavy articles but may be entirely omitted without sensible loss of advantage in the case of light articles. Where steam is employed, lime highly hygroscopic may be introduced into the muffle to facilitate the formation of the rust proofing surface by catalytic action. Naphtha or other hydrocarbon in small quantities may be injected with the steam to impart a black color to the surface.

A suitable apparatus for carrying out the invention is illustrated diagrammatically in the accompanying drawings, in which,

Figure 1 is a vertical section of the heating apparatus; and Fig. 2 a sectional plan with the muffle removed.

In the form shown, which may be variously modified without departing from my invention, the apparatus comprises a muffle chamber 10 of fire-brick or other suitable refractory material, within which the article 11, which is under treatment, is placed. This muffle is heated to the required temperature by any suitable means, burners 12 being shown projecting into the space beneath the muffle. The products of combustion pass up around the muffle and escape at the outlet 13 at the top of the casing 14.

of fire-brick and asbestos. Beneath the muffle and adjacent the burners I arrange for the sake of economy a steam box 15 in which the steam coming from any suitable source through the pipe 16 is superheated before introduction through the pipe 17 into the muffle chamber. A valve 18 controls the inlet for the steam. On the opposite side of the furnace I have arranged a retort 19 in which are placed the substances comprising the rust proofing material. The latter is fused by the heat from the burners and the fumes pass up from the retort through the pipe 20 to the muffle chamber. A door 21 is provided for the retort chamber through which the chemicals may be introduced.

Where treatment by steam is not to be used in any particular case the articles to be treated are first heated by placing them in the muffle and starting the burners. As soon as a suitable temperature has been secured in the muffle chamber the rust proofing material is placed in the chemical retort, where it is rapidly heated to a temperature of 1400° F. or higher and the fumes rise from the fused material to the muffle chamber and rapidly condense upon the articles therein. If the articles are to be first heated by steam, however, the cock 18 is opened and the steam passing through the steam box 15 enters the muffle chamber superheated to a temperature of 1400° F. or above. After the steam has been in contact with the articles a sufficient length of time, the cock 18 is closed and the temperature of the chamber soon drops to 1200° F. or less. The chemicals are then introduced into the retort 19 and after the fumes thereof have filled the muffle for the desired length of time, the heat is cut off and the muffle permitted to cool sufficiently to allow the withdrawal of the articles under treatment.

As examples of non-corrodible material suitable for use in this process, I may use, (1) tannic acid, an oleaginous material and a non-corrodible material such as zinc or an oxid of such metal; or (2) a pure metal such as zinc or lead, or (3), substantially solid hydrocarbon such as coal tar or pitch. The first of these materials gives a good coating a dark gray color; the second gives also a good coating a blue color, while the third gives a black coating of the very highest quality.

Before the treatment, the metal is washed perfectly clean, as usual, in rust proofing processes. After the goods are taken out of the muffle they are cooled to about 100° F. and greased with vaseline and cleaned so as

to give them a good polish and an attractive 60 appearance.

I claim as my invention:—

1. The method of protecting iron or steel which comprises the step of subjecting the same to the action of the fumes of a fused, 65 non-corrodible metalliferous substance in a closed chamber, the temperature of the article during the treatment thereof with said fumes being maintained above the fusing and below the fuming temperature of said 70 substance whereby a non-corrodible deposit is formed in a liquid state upon said article during treatment, substantially as described.

2. The method of protecting iron or steel which comprises the step of subjecting the 75 same to the action of the fumes of a fused, non-corrodible metalliferous substance, comprising zinc, in a closed chamber, the temperature of the article during the treatment thereof with said fumes being maintained 80 above the fusing and below the fuming temperature of said substance whereby a non-corrodible deposit is formed in a liquid state upon said article during treatment, substantially as described. 85

3. The method of protecting iron or steel which consists in subjecting the same to the action of steam and then subjecting the same to the action of the fumes of a fused, non-corrodible metalliferous substance in a closed 90 chamber, the temperature of the article during the treatment thereof with said fumes being maintained above the fusing and below the fuming temperature of said substance whereby a non-corrodible deposit is 95 formed in a liquid state upon said article during treatment, substantially as described.

4. The method of protecting iron or steel which consists in subjecting the same to the action of steam and then subjecting the same 100 to the action of the fumes of a fused, non-corrodible metalliferous substance, comprising zinc, in a closed chamber, the temperature of the article during the treatment thereof with said fumes being maintained 105 above the fusing and below the fuming temperature of said substance whereby a non-corrodible deposit is formed in a liquid state upon said article during treatment, substantially as described. 110

In testimony whereof I have signed my name to this specification, in the presence of two subscribing witnesses.

AUGUSTO BONTEMPI.

Witnesses:

H. D. LUCE,  
Wm. R. SWAN.